

H. B. SLATER.

PROCESS OF MAKING A LEACHING SOLUTION FOR EXTRACTION OF METALS FROM THEIR ORES.

APPLICATION FILED JULY 28, 1915.

1,195,617.

Patented Aug. 22, 1916.



Inventor:

Henry Byron Slater.

by  
Arthur D. Knight  
Atty

# UNITED STATES PATENT OFFICE.

HENRY BYRON SLATER, OF LOS ANGELES, CALIFORNIA.

## PROCESS OF MAKING A LEACHING SOLUTION FOR EXTRACTION OF METALS FROM THEIR ORES.

1,195,617.

Specification of Letters Patent. Patented Aug. 22, 1916.

Application filed July 28, 1915. Serial No. 42,342.

To all whom it may concern:

Be it known that I, HENRY BYRON SLATER, a citizen of the United States, residing at Los Angeles, in the county of Los Angeles and State of California, have invented a new and useful Process of Making a Leaching Solution for Extraction of Metals from Their Ores, of which the following is a specification.

10 This invention relates to the production of a solution containing chlorin in active form, for extraction of copper or other metals from ores containing same, and particularly to the production of a solution containing ferric chlorid and sodium chlorid, together with free chlorin and oxidation products thereof.

20 The main object of the present invention is to provide for the production of such a solution at minimum expenditure for apparatus and for operation thereof.

25 The accompanying drawing illustrates an apparatus suitable for carrying out my invention, said drawing being a vertical section of such apparatus.

30 The apparatus shown in the drawing comprises an electrolytic cell, consisting of a container or cell 1, having a diaphragm 2 of suitable porous material, such as asbestos cloth and electrodes 3 and 4 suitably supported in the respective compartments 5 and 6 of said cell, on opposite sides of said diaphragm. Said electrodes may be of any suitable material, for example, carbon, and 35 are connected to the wires 7 and 8 of a direct current supply circuit of suitable voltage.

40 My process consists essentially in subjecting a solution containing ferrous chlorid and sodium chlorid to electrolysis in the anode compartment of an electrolytic cell, until all the ferrous chlorid has been converted into ferric chlorid by the action of the chlorin set free at the anode and then continuing 45 the electrolysis until free chlorin and hypochlorous acid are produced in considerable amount, by the liberation of a further amount of chlorin at the anode, and regulating or controlling the diffusive communication 50 between the cathode and anode compartments, by means of the permeable diaphragm between said compartments, so as to produce the amount of hypochlorous acid

or chlorin oxidation product required for the leaching operation.

55 The process may be carried out as follows, in preparing a solution to be used for extraction of copper from its ores: A solution containing say one per cent. of ferrous chlorid, and ten per cent. of sodium chlorid, 60 is passed into the anode compartment of the electrolytic cell, and any suitable solution placed in the cathode compartment, for example, a ten per cent. solution of sodium chlorid. Current is then passed through 65 the cell, with the result that chlorin is set free at the anode by the electrolysis of the sodium chlorid, and sodium hydroxid is produced in the cathode compartment. The primary action of the chlorin set free in this 70 manner is to convert the ferrous chlorid to ferric chlorid, and in processes of this nature it is usual to stop the electrolysis as soon as all of the ferrous chlorid has been converted in this manner to ferric chlorid. In my 75 present process, however, I continue the electrolysis after all of the ferrous chlorid has been converted to ferric chlorid, and thereby produce a solution containing, in addition to the ferric chlorid, a considerable 80 amount of free chlorin and also containing a considerable amount of oxidation products of chlorin, and particularly hypochlorous acid, and the solution so produced is of especial advantage in leaching certain kinds 85 of ores, particularly ores containing copper sulfid.

8 In my Patent No. 1,066,855, dated July 8, 1913, a process was described in which hypochlorous acid was produced by electrolysis of a similar solution in the anode compartment of an electrolytic cell by adding electrolytic products from the cathode compartment to the anode compartment after all 90 of the ferrous chlorid was converted to ferric chlorid. According to my present invention the hypochlorous acid is produced by reaction of the chlorin set free at the anode, with substances present in the anode compartment itself and without addition of 100 cathode products except in so far as they may pass automatically to the anode compartment, by diffusion or by migration through the diaphragm from the cathode compartment. The present invention is, 105 therefore, directed particularly to the pro-

duction of hypochlorous acid in the anode compartment by the operation of the cell itself, without requiring bodily transfer of a portion of the cathode solution to the 5 anode compartment.

I have found that by subjecting a solution such as above described to electrolysis under the stated conditions, and by maintaining a suitable permeability of the dia- 10 phragm between the compartments of the electrolytic cell, that it is possible to produce, by the action of the liberated chlorin in the anode compartment on substances present in said compartment, including 15 cathode products diffusing through the dia- phragm, sufficient amount of hypochlorous acid and other chlorin-oxidation products to render the resulting solution extremely effective as a leaching agent for extracting 20 copper or other metals from ores thereof. The permeability of the diaphragm may be controlled or determined by its thickness, or by the closeness of its texture, the dia- phragm being constructed or formed so as 25 to present the proper texture and thickness required to give the needed permeability, without permitting such excessive passage of the cathode products, such as sodium hy- droxid, to the anode compartment as would 30 result in interference with effective electrol- ysis.

One way in which the hypochlorous acid may be produced in the anode compartment is by reaction of the free chlorin with the 35 water, or with the hydrogen and hydroxyl ions, present in said compartment, this re- action being represented by the following equation:



Another way in which the hypochlorous acid may be produced is by reaction of the free chlorin with the hydroxyl ions migrating from the cathode compartment into the 45 anode compartment, this reaction being represented by the equation:



Another mode of formation of the hypo- 50 chlorous acid is by the action on the anode solution, of sodium hydroxid diffusing thereinto from the cathode compartment, this reaction being represented by the equations:



The amount to which these reactions may take place, particularly the reactions involv- 60 ing the action of hydroxyl ions migrating through the permeable diaphragm and the action of sodium hydroxid diffusing through said diaphragm, may be regulated and determined by the permeability of such dia- phragm, so that by suitably modifying such

permeability any required amount of hypo- chlorous acid may be obtained.

In order to further regulate or control the amount of hypochlorous acid produced in the anode compartment, so as, for ex- 70 ample, to permit of further and closer regulation during operation of the cell, I may vary the diffusive head through the dia- phragm, either by modifying the concentra- 75 tion of the sodium hydroxid in the cathode compartment, or by maintaining and regu- lating a hydrostatic head between the com- 80 partments. Thus, the greater the concentra- 85 tion of the sodium hydroxid in the cathode compartment, and the greater the hydro- static head between the anode and cathode compartments, the greater will be the rate 90 of diffusion of sodium hydroxid through a diaphragm of given permeability, so that by suitably modifying the said concentra- 95 tion and the said hydrostatic head any desired closeness of regulation of the hypochlorous acid production may be obtained. These objects may be obtained by regulating the flow of sodium chlorid solution to the 90 cathode compartment by a valved inlet 9 and regulating its outflow by a valved out- 95 let 10, and by regulating the height of liquid in the anode compartment by valved inlet and outlet connections 11, and 12. 95

In place of sodium chlorid, any other alkali metal chlorid or alkaline earth metal chlorid may be used in the solution as a leaching agent and as a source of chlorin in the electrolytic operation, and the term 100 "sodium chlorid" as herein used includes any of such equivalent chlorids.

What I claim is:

1. The process of producing a solution for 105 extracting metals from their ores, which consists in subjecting a solution of ferrous chlorid and sodium chlorid to electrolysis in the anode compartment of an electrolytic cell; and simultaneously subjecting a solution of sodium chlorid to electrolysis in the 110 cathode compartment of such cell, maintaining separation of said compartments by a diaphragm of sufficient permeability to enable diffusion of cathode products from the cathode compartment to the anode compart- 115 ment, and continuing electrolysis after all of the ferrous chlorid has been converted to ferric chlorid, so as to produce hypochlorous acid by reaction of the chlorin set free in the anode compartment with cathode prod- 120 ucts diffusing from the cathode compart- ment.

2. The process of producing a leaching solution for extracting metals from their 125 ores, which consists in subjecting a solution of ferrous chlorid and sodium chlorid to electrolysis in the anode compartment of an electrolytic cell, simultaneously subjecting a solution containing sodium chlorid to elec- 130 trolysis in the cathode compartment of said

cell, continuing the electrolysis until all the ferrous chlorid is converted to ferric chlorid, and then continuing the electrolysis so as to liberate a further quantity of chlorin, and controlling the products of electrolysis by maintaining a diaphragm of such permeability between the compartments as to permit sufficient passage of cathode products to the anode compartment to produce, by reaction with the free chlorin therein chlorin oxidation products to the extent desired in the leach, and further controlling the production of chlorin oxidation products by maintaining and regulating a hydrostatic head between said compartments.

3. The process of producing a leaching solution for extracting metals from their ores, which consists in subjecting a solution of ferrous chlorid and sodium chlorid to electrolysis in the anode compartment of an electrolytic cell, simultaneously subjecting a

solution containing sodium chlorid to electrolysis in the cathode compartment of said cell, continuing the electrolysis until all the ferrous chlorid is converted to ferric chlorid, 25 and then continuing the electrolysis so as to liberate a further quantity of chlorin, and controlling the products of electrolysis by maintaining a diaphragm of such permeability between the compartments as to permit sufficient passage of cathode products to the anode compartment to produce, by reaction with the free chlorin therein, chlorin oxidation products to the extent desired in the leach, and further controlling the production of chlorin oxidation, by regulating the concentration of cathode products in the cathode compartment.

In testimony whereof I have hereunto set my hand, at Los Angeles, California, this 40 21st day of July 1915.

HENRY BYRON SLATER.